

[54] FOGGED, DIRECT-POSITIVE SILVER HALIDE PHOTOGRAPHIC MATERIAL CONTAINING A RHODIUM SALT DESENSITIZER AND A BISPYRAZOLONE DYE STABILIZER

[75] Inventors: Tetsuo Furuya, Ashigara; Hidehiko Ishikawa; Hideo Kanisawa, both of Odawara, all of Japan

[73] Assignee: Konishiroku Photo Industry Co., Ltd., Tokyo, Japan

[22] Filed: Apr. 26, 1973

[21] Appl. No.: 354,842

[30] Foreign Application Priority Data

May 4, 1972 Japan ..... 47-43679

[52] U.S. Cl. .... 96/101, 96/107, 96/108, 96/109, 96/125, 96/139, 96/140

[51] Int. Cl. .... G03c 1/28, G03c 1/34, G03c 1/36

[58] Field of Search ..... 96/107, 108, 109, 101, 96/125, 139, 140

[56]

References Cited

UNITED STATES PATENTS

|           |        |                      |        |
|-----------|--------|----------------------|--------|
| 2,717,833 | 9/1955 | Wark .....           | 96/108 |
| 3,576,636 | 4/1971 | Matsui et al. ....   | 96/101 |
| 3,656,961 | 4/1972 | Hayakawa et al. .... | 96/108 |
| 3,738,846 | 6/1973 | Kamano et al. ....   | 96/101 |

Primary Examiner—Ronald H. Smith

Assistant Examiner—Won H. Louie, Jr.

Attorney, Agent, or Firm—Bierman & Bierman

[57]

ABSTRACT

A direct - positive light - sensitive silver halide material containing fogged silver halide grains and a rhodium salt as a desensitizer to increase the reversal speed, which material comprises a bis-pyrazolone dye having an absorption maximum in the range from 590 to 690 mu, said bis-pyrazolone dye having a methine chain connecting two pyrazolone nuclei thereof, said methine chain consisting of 5 unsubstituted methine groups.

2 Claims, No Drawings

**FOGGED, DIRECT-POSITIVE SILVER HALIDE  
PHOTOGRAPHIC MATERIAL CONTAINING A  
RHODIUM SALT DESENSITIZER AND A  
BISPYRAZOLONE DYE STABILIZER**

This invention relates to a light-sensitive silver halide photographic material. More particularly, the invention pertains to a solarization type direct-positive light-sensitive material.

Generally, a direct-positive light-sensitive material utilizing Harschel effect (a so-called Harschel type direct-positive light-sensitive material) and a direct-positive light-sensitive material utilizing solarization (a so-called solarization type direct-positive light-sensitive material) have been known as typical direct-positive light-sensitive materials.

It is well known that the solarization type direct-positive light-sensitive material is of such a type that moderately pre-fogged nuclei effect subtraction due to excess exposure to give a direct-positive image, and hence is essentially different from the Harschel type direct-positive light-sensitive material which utilizes the phenomenon that pre-fogged nuclei effect subtraction due to red light or infrared light.

Ordinarily, the polarization type direct-positive light-sensitive material has moderately been pre-fogged by application of light or by adoption of such chemical means as using a fogging agent, and it is well known that subtraction of the fog is promoted by use of a desensitizer to increase the reversal speed of the light-sensitive material. It is also well known that when a rhodium salt is used as the desensitizer in the above case, there is obtained a polarization type direct-positive light-sensitive material which is relatively high in speed.

Despite of its relatively high in speed, however, the solarization type direct-positive light-sensitive material containing a rhodium salt as the desensitizer is low in safeness to darkroom light and hence is inconvenient in

handling. This tendency is particularly marked when the said light-sensitive material has been optically sensitized by incorporation of a sensitizing dye or the like and has been made higher in speed by interaction of said dye with the rhodium salt. Consequently, the light-sensitive material is deteriorated in safeness to a darkroom light of orange to red color, which is ordinarily used in a darkroom, with the result that the density is lowered.

10 A principal object of the present invention is to provide a solarization type direct-positive light-sensitive material which is not only high in speed but also has enhanced safeness to darkroom light.

As the result of extensive studies, we have found that

15 the above-mentioned object can successfully be accomplished by incorporating into at least one of the photographic layers, e.g., protective layer, inter layer, emulsion layer, sub layer or backing layer, of a solarization type direct-positive light-sensitive material containing a rhodium salt as a desensitizer, a certain dye in a proportion of 1 to 500 mg. per 100 cm<sup>2</sup> of the light-sensitive material.

20

The dye used in the present invention is required to have an absorption maximum in the range from 590 to 25 690  $\mu\mu$ . In case a dye having an absorption maximum

30 35 390 m. $\mu$ . In case a dye having an absorption maximum exceeding the said range has been used, the light-sensitive material is insufficient in safeness to darkroom light, while in case a dye having an absorption maximum smaller than said range has been used, the light-sensitive material gives an image which is unsatisfactory in photographic property. The amount of the dye used in the present invention should be in the range from 1 to 500 mg. per 100 cm<sup>2</sup> of the effective area of the light-sensitive material. If the amount of the dye is out of said range, either the photographic property or the safeness to darkroom light is unsatisfactory.

Typical examples of the dye used in the present invention are shown below, but dyes usable in the present invention are not limited to these.

40





The dye used in the present invention is preferably such that it is water-soluble and leaves no stains after development. The dye is dissolved in a proper solvent such as water, methanol, ethanol or acetone, and then incorporated into any of the photographic layers of a polarization type direct-positive light-sensitive material. In this case, the dye is preferably incorporated into the protective layer or the like layer which is upper than the light-sensitive layer. If necessary, however, the dye is incorporated into the backing layer, sub layer or the like layer which is lower than the light-sensitive layer. In case the dye has no influence on photographic properties of the light-sensitive material, it may be incorporated into the light-sensitive layer or into the inter layer or the like layer adjacent to the light-sensitive layer. The amount of the dye to be incorporated is 1 to 500 mg., preferably about 5 to 50 mg., per 100 cm<sup>2</sup> of the effective area of the light-sensitive material.

The polarization type direct-positive light-sensitive material according to the present invention which is prepared in the above manner not only has excellent speed and safeness to darkroom light but also is excellent in other photographic properties.

The rhodium salt used in the present invention is a water-soluble rhodium salt such as rhodium chloride or rhodium bromide which is used as a desensitizer. Generally, the rhodium salt is added at the time of emulsification or physical ripening of silver halide, and is ordinarily used in a proportion within the range from about 0.5 to 400 mg. per mole of silver halide. The silver halide may be any of such silver halides as silver chlorobromide, silver bromide, silver chloroiodobromide and silver iodobromide, and the silver halide emulsion may be prepared according to any of acid process, neutral process and ammonia process. In this case, gelatin is ordinarily used as the protective colloid. Alternatively, however, other hydrophilic protective colloid such as albumin, polyvinyl alcohol and the like may be used either singly or in admixture with gelatin or in the form of a mixture of two or more.

The silver halide emulsion is fogged according to an ordinary procedure with a reducing agent such as stannous chloride, formaldehyde or thiourea dioxide, or with a salt of a metal high in potential than silver such as potassium chloroaurate, or with a combination of the two. Ordinarily, the reducing agent is used in a pro-

portion of about 0.05 to 400 mg., and the salt of a metal higher in potential than silver is used in a proportion of about 0.5 to 100 mg., per mole of silver halide.

The light-sensitive material according to the present invention may contain various photographic additives, e.g., a hardener such as formaldehyde, glyoxal or such substituted fatty acid as mucobromic acid, an extender such as saponin, a stabilizer, couplers, etc. More pref-

The thus prepared sample was allowed to stand with the emulsion side up and at a distance of 1 m. under a 20W darkroom lamp with a red filter for such a period of time as shown in Table 1. Thereafter, the sample was subjected to ordinary development (using, for example, the D-72 developer produced by Kodak Co.) and then measured in density to obtain the results as set forth in Table 1.

Table 1

| Dye          | Amount per 100 cm <sup>2</sup> | Reversal speed (relative value) | Density                     |                             |                             |                              |                              |
|--------------|--------------------------------|---------------------------------|-----------------------------|-----------------------------|-----------------------------|------------------------------|------------------------------|
|              |                                |                                 | Allowed to stand for 0 min. | Allowed to stand for 3 min. | Allowed to stand for 5 min. | Allowed to stand for 10 min. | Allowed to stand for 20 min. |
| Compound (1) | 60 mg.                         | 100                             | 2.68                        | 2.65                        | 2.60                        | 2.55                         | 2.41                         |
| Compound (3) | 150 mg.                        | 92                              | 2.72                        | 2.70                        | 2.69                        | 2.67                         | 2.63                         |
| Compound (7) | 120 mg.                        | 90                              | 2.63                        | 2.63                        | 2.61                        | 2.59                         | 2.55                         |
|              |                                | 95                              | 2.65                        | 2.65                        | 2.64                        | 2.62                         | 2.60                         |

erably, the light-sensitive material is optically sensitized with any of such spectral sensitizers as cyanine and merocyanine dyes.

The present invention is illustrated in further detail below with reference to examples, but the scope of the invention is not limited to the examples.

### EXAMPLE 1

|                            |     |     |  |  |
|----------------------------|-----|-----|--|--|
| Liquid I:                  |     |     |  |  |
| Gelatin                    | 20  | g.  |  |  |
| Citric acid                | 0.4 | g.  |  |  |
| Water                      | 400 | cc. |  |  |
| Liquid II:                 |     |     |  |  |
| Silver nitrate             | 40  | g.  |  |  |
| Water                      | 400 | cc. |  |  |
| Liquid III:                |     |     |  |  |
| Sodium chloride            | 14  | g.  |  |  |
| Potassium bromide          | 12  | g.  |  |  |
| Rhodium chloride solution* | 8   | cc. |  |  |
| Water                      | 90  | cc. |  |  |
| Liquid IV:                 |     |     |  |  |
| Gelatin                    | 70  | g.  |  |  |
| Potassium iodide           | 0.2 | g.  |  |  |
| Water                      | 300 | cc. |  |  |

\*A solution of 0.1 g. of  $\text{RhCl}_3 \cdot 4\text{H}_2\text{O}$  in 100 cc. of a 25% aqueous sodium chloride solution.

The liquid II was added at 50°C. to the liquid I, and then the liquid III was added to the resulting mixture with stirring to prepare an emulsion. The emulsion was ripened at 50°C. for 40 minutes and then charged with the liquid IV. After 10 minutes, the emulsion was adjusted to a pH of 8.8 by addition of alkali, and 5 cc. of a 4 percent formaldehyde solution was added thereto. After fogging by incubation at 50°C. for 15 minutes, the emulsion was neutralized to a pH of 6.0 by addition of acid. Subsequently, the emulsion was incorporated with an ortho-sensitizing dye 3,3'-9-triethyloxacarbocyanine iodide, a hardener and a surface active agent, coated on a transparent support and then dried to prepare a sample.

### EXAMPLE 2

|                           |     |     |  |            |
|---------------------------|-----|-----|--|------------|
| Liquid I:                 |     |     |  |            |
| Gelatin                   | 16  | g.  |  |            |
| Water                     | 110 | cc. |  |            |
| Potassium bromide         | 34  | g.  |  |            |
| Potassium iodide          | 0.7 | g.  |  |            |
| Rhodium chloride solution | 1.5 | cc. |  |            |
| Liquid II:                |     |     |  |            |
| Silver nitrate            | 48  | g.  |  |            |
| Water                     | 400 | cc. |  |            |
| Ammonia water             |     |     |  | Equivalent |

The liquid II was added to the liquid I to prepare an emulsion. The emulsion was ripened at 40°C. for 10 minutes and then neutralized to a pH of 6.5 by addition of acid. Subsequently, the emulsion was washed with water, stirred at 50°C. for 10 minutes together with 12 g. of gelatin and then properly fogged with a mixture of a reducing agent and a gold compound. One half of the thus treated emulsion was incorporated with a hardener and a surface active agent to form an emulsion (A), and the other half of the emulsion was incorporated with an ortho-sensitizing dye 3,3'-9-triethyloxacarbocyanine iodide, a hardener and a surface active agent. Each of the emulsions (A) and (B) was coated on a transparent support. Subsequently, a protective layer-forming solution incorporated with each of such dyes as shown in Table 2 was coated on the resulting emulsion layer and then dried to prepare a sample. The thus prepared sample was treated in the same manner as in Example 1 and then measured in density to obtain the results as set forth in Table 2.

Table 2

| Emul-sion | Dye          | Amount per 100 cm <sup>2</sup> | Reversal speed (relative value) | Density                     |                             |                             |                              |                              |
|-----------|--------------|--------------------------------|---------------------------------|-----------------------------|-----------------------------|-----------------------------|------------------------------|------------------------------|
|           |              |                                |                                 | Allowed to stand for 0 min. | Allowed to stand for 3 min. | Allowed to stand for 5 min. | Allowed to stand for 10 min. | Allowed to stand for 20 min. |
| A         | —            | —                              | 20                              | 4.07                        | 4.02                        | 3.95                        | 3.88                         | 3.56                         |
| A         | Compound (2) | 25 mg.                         | 19                              | 4.08                        | 4.08                        | 4.07                        | 4.06                         | 4.05                         |
| B         | —            | —                              | 100                             | 4.01                        | 3.75                        | 3.39                        | 3.03                         | 2.05                         |
| B         | Compound (2) | 25 mg.                         | 96                              | 4.02                        | 4.01                        | 3.98                        | 3.85                         | 3.70                         |
| B         | Compound (6) | 30 mg.                         | 95                              | 4.00                        | 4.00                        | 3.95                        | 3.83                         | 3.65                         |
| B         | Compound (4) | 35 mg.                         | 93                              | 3.99                        | 3.95                        | 3.89                        | 3.80                         | 3.71                         |
| B         | Compound (5) | 50 mg.                         | 90                              | 4.03                        | 4.01                        | 4.00                        | 3.95                         | 3.88                         |
| B         | Compound (8) | 30 mg.                         | 98                              | 4.01                        | 4.00                        | 3.98                        | 3.90                         | 3.95                         |

From Table 2, it is understood that each sample according to the present invention is scarcely degraded in density even when allowed to stand under a darkroom light for a long period of time.

What we claim is:

1. A direct-positive light-sensitive silver halide material containing fogged silver halide grains and a rhodium salt as a desensitizer to increase the reversal speed, which material comprises a bis-pyrazolone dye having an absorption maximum in the range from 590 to 690 m $\mu$ , which dye is present in an amount of 1 to 500 mg. per 100 cm $^2$  of the effective area of said sensitive material, said bis-pyrazolone dye having a methine chain connecting two pyrazolone nuclei thereof, said methine chain consisting of 5 unsubstituted methine groups.

2. A direct-positive light-sensitive material according to claim 1, wherein said bis-pyrazolone dye is selected from the following compounds:



\* \* \* \* \*